

## UNITED STATES PATENT OFFICE

2,130,570

PROCESS FOR FULLING OR FELTING WOOL  
OR HAIR

Anton Volz, Ludwigshafen-on-the-Rhine, Germany, assignor, by mesne assignments, to Hall Laboratories Inc., Pittsburgh, Pa.

No Drawing. Application July 27, 1936, Serial No. 92,923. In Germany August 1, 1935

9 Claims. (Cl. 26—19)

The working up of wool and hair to a compact felted layer is effected by means of fulling or milling operations.

The milling or fulling is carried out with mechanical treatment of the material being felted, if necessary in the hot, in alkaline or acid fulling bath. Alkaline fulling agents heretofore have been prepared with addition of alkalies, such as soda and potash, and acid fulling agents with addition of inorganic and organic acids.

The employment of these fulling agents requires special experience and very easily leads to a mechanical and chemical injury of the material being fulled, particularly when these fulling agents are employed in concentrations which yield an optimum fulling effect.

The surprising observation has now been made that by means of water-soluble salts of those phosphoric acids which are poorer in water than orthophosphoric acid, that is to say, contain less constitutional water than orthophosphoric acids (such as pyro- and meta-phosphoric acids), a substantial improvement in the fulling action is produced, and in fact both in the case of fulling in the greasy or dirty condition as well as in the case of neutral to alkaline fulling of pre-washed goods and also in the case of acid fulling of pre-washed goods.

This improvement is a specific enhancement of the fulling action with maintenance of the usual additions at the same time which brings about a finer and more compact felt formation and a better removal of the fat substances and dirt from the goods. This better fulling action is assisted by the lime-binding, magnesia-binding and iron-binding action of anhydrous phosphates, it being particularly necessary to avoid these disturbing metals or their carbonates or fatty acid salts settling in the goods.

The above-mentioned phosphates offer the advantage that a better felt is produced in a shorter time, with lower alkalinity, that is to say with maximum preservation of the fibres and best maintenance of the weight.

The goods run more easily in the presence of phosphate solutions and are softer and more extensible under the fulling or milling members and mechanically are impaired to a considerably less extent; more particularly the felting in of fulling marks is avoided. Fats which are difficult to saponify are saponified more rapidly so that the additional addition of soap can be dispensed with.

Pre-washed goods can be fulled or milled with suitable phosphate mixtures without soap and

without alkali, and in fact in alkaline, neutral and acid medium.

## Example of fulling or milling in the greasy or dirty condition

Two pieces of goods weighing altogether 50 kg. are introduced on to the milling cylinder and, corresponding to the dirt content, soda lye of 2° Baumé, which contains in addition 10 g. sodium hexametaphosphate and 5 g. sodium pyrophosphate per litre, is poured on. A strong froth immediately forms and the goods begin to felt uniformly.

## Example of the fulling or milling of pre-washed goods

The goods are washed at 40° C. with 2-3 g. per litre of calcined soda and 1 g. per litre of a mixture of sodium hexametaphosphate and sodium pyrophosphate. The washing takes about ½ hour and then the goods are rinsed. The material is then treated on the fulling or milling machine with a sodium pyrophosphate solution containing 40 g. per litre, the quantity being such that the goods do not become too wet.

Instead of sodium pyrophosphate, polyphosphates or mixtures of sodium hexametaphosphate with soap or with acids can also be used, and in fact in concentrations of 2-100 g. per litre of liquor.

After all fulling or milling rinsing is effected, if desired with addition of 1 g. per litre of a mixture of sodium hexametaphosphate with sodium pyrophosphate.

## Example for acid fulling

The pre-cleaned goods are soaked in a 5% solution of a mixture of acid pyrophosphate and metaphosphate, (pH 4.04) and fulled on the machine.

## Example for neutral fulling

The pre-cleaned goods are fulled on the machine with an 8% solution of a mixture of tetra-sodium pyrophosphate and metaphosphate which has been adjusted to pH 7.0, so much of this solution being poured on to the goods that the latter proceeds sufficiently moist, in general twice to three times the weight of the goods being used.

## Example for alkaline fulling with agents which promote felting

The carded yarn goods oiled with olein are treated, per hank, with 2 buckets (=20 litres) of a solution of 15-20 g. per litre of soda and 5-10 g. per litre of sodium polyphosphate ( $\text{Na}_5\text{P}_4\text{O}_{13}$ ),

whereupon the goods are fulled as usual until they show the requisite contraction in width and length.

5 If a material is fulled for 30 minutes at 25° on the machine in a 2.5% fulling solution which contains

1. Soda (pH=11.6)
2. Neutral pyrophosphate (pH=9.6)
3. A mixture of pyrophosphate and metaphosphate (pH=8.8)
4. Metaphosphate (pH=6.65)
5. A mixture of acid pyrophosphate and metaphosphate (pH=4.04)
6. Polyphosphate (pH=7.5)

15 then in the case of the substance fulled with soda a pronounced streak formation occurs and the initial fulling is inferior. The initial fulling in the case of all anhydrous phosphates is uniform 20 and the fulled product of a very fine full feel.

20 The use of these salts as fulling agents affords the further advantage that with them both alkaline, neutral as well as acid fulling baths can be prepared and that also in addition the pH value 25 can be varied during the fulling within the wide limits. As a result it is possible to take into account to a maximum degree the preservation or protection of the fibre and colour.

When using these salts known agents which 30 promote the formation of felt and which do not impair the fibre can be employed as well in addition.

What I claim is:

35 1. The method of fulling or felting wool or hair in alkaline, neutral or acid medium which consists in employing as fulling agent at least one water-soluble salt of a phosphoric acid containing less water than orthophosphoric acid.

40 2. The method of fulling or felting wool or hair in alkaline, neutral or acid medium which consists in employing as fulling agent a mixture of alkali metal hexametaphosphate and alkali metal pyrophosphate.

3. The method of fulling or felting wool or hair in alkaline, neutral or acid medium which consists in employing as fulling agent a water-soluble polyphosphate together with a water-soluble metaphosphate.

4. The method of fulling or felting wool or hair in alkaline, neutral or acid medium which consists in employing as fulling agent a mixture of alkali metal hexametaphosphate and soap.

5. The method of fulling or felting wool or hair 10 in alkaline, neutral or acid medium which consists in employing as fulling agent a mixture of alkali metal hexametaphosphate and acid.

6. The method of fulling or felting wool or hair 15 in alkaline, neutral or acid medium which consists in fulling the said material with the aid of at least one water-soluble salt of a phosphoric acid containing less constitutional water than orthophosphoric acid, and rinsing the fulled goods in water containing a small quantity of alkali metal hexametaphosphate and alkali metal pyrophosphate.

7. The method of fulling or felting wool or hair 20 in alkaline, neutral or acid medium which consists in employing as fulling agent at least one water-soluble salt of a phosphoric acid containing less constitutional water than orthophosphoric acid in conjunction with other known agents which promote felting.

8. The method of fulling or felting wool or hair 30 which consists in treating the material with soda lye containing a small amount of alkali metal hexametaphosphate and alkali metal pyrophosphate.

9. The method of fulling or felting wool or hair 35 consisting in washing the material with an aqueous solution containing calcined soda, alkali metal hexametaphosphate and alkali metal pyrophosphate, and then fulling it with a solution containing alkali metal pyrophosphate.

40 ANTON VOLZ.